

## UNITED STATES PATENT OFFICE

CORNELL H. CORDIE, OF WILMINGTON, DELAWARE, AND WILLARD DE C. CRATER, OF SUCCASUNNA, NEW JERSEY, ASSIGNEES TO HERCULES POWDER COMPANY, OF WILMINGTON, DELAWARE, A CORPORATION OF DELAWARE

## METHOD FOR PRODUCING EXPLOSIVE

No Drawing.

Application filed September 25, 1929. Serial No. 395,194.

This invention relates to a method for the production of an explosive, more particularly adaptable for use in connection with the production of dynamites, gelatins and the like having a low freezing point, or which will not freeze at such low temperatures as ordinarily prevail in temperate climates.

Heretofore an explosive for incorporation into dynamites, gelatins, etc., for the production of an explosive having a low freezing point and involving nitroglycerine, nitrodi-glycerine, dinitroglycol and the like in admixture with a nitrotoluene, as dinitrotoluene, has been known. However, in the production of such explosive heretofore, the glycerine, glycol or the like and the toluene have been separately nitrated and the nitrated products admixed for the production of the desired explosive.

While the nitration of glycerine, glycol, or the like, does not present a difficult problem, nitration of toluene is more complicated and is troublesome to a substantial degree. For example, in the manufacture of dinitrotoluene, special apparatus is required and the nitrating acids, after separation from the dinitrotoluene, carry a substantial quantity thereof in solution, which causes considerable difficulty in effecting denitration of the spent acids.

Now, in accordance with this invention, it has been found that an explosive of the type desired, that is to say, comprising a mixture of nitrated glycerine, glycol or the like and nitrated toluene, may be produced readily and without difficulty by effecting the nitration of the glycerine, glycol, or the like, and the toluene by a combined process, rather than separately as heretofore.

In proceeding in accordance with the method embodying this invention, not only is the necessity for separate apparatus obviated, but the difficulty and trouble incident to the separate manufacture of the nitrated toluene are avoided. At the same time, the nitrated mixture produced is stable after the usual purification treatment, may be made to contain a desirable quantity of nitrated toluene and is usable directly in the manufacture of dyna-

mites, gelatins, and the like, having a low freezing point.

As illustrative of the practical adaptation of the method involving this invention, for example, the usual mixture of glycerine and diglycerine is run into a nitrator of usual construction containing a usual nitrating mixture until about 30-40% of the charge has been added, after which, and while continuing the introduction of the glycerine-diglycerine mixture into the nitrator, toluene is simultaneously introduced into the nitrator. The total charge of toluene is desirably added by the time (say) 60-70% of the glycerine-diglycerine mixture has been run or introduced into the nitrator. After the toluene is added, the balance of the charge of the glycerine-diglycerine mixture is introduced into the nitrator. During the addition of the glycerine and of the toluene the temperature of the nitrating mixture is controlled to obtain maximum yield. The nitrated products are subjected to washing with water and alkaline solution, as is usual for the purification and stabilization of the product.

As a more specific example of the practical adaptation of the method involving this invention, 500 parts of a nitrating mixture, comprising, for example,  $H_2SO_4$ , 52.60%;  $HNO_3$ , 46.36%;  $HNOSO_4$ , .95%;  $H_2O$ , .09%; are placed in a nitrator of usual construction. The nitrating mixture is cooled to a temperature of (say) about 36° F. and about 100 parts of a glycerine-diglycerine mixture slowly added. After about one-third or (say) 30-40% of the glycerine-diglycerine mixture has been added to the nitrator, 7 parts of toluene are added separately during the addition of a further third or (say) 30-40% of the glycerine-diglycerine mixture, and, finally, the remaining third or (say) 30-40% of the glycerine-diglycerine mixture is added. When nitration is completed, the nitrated products are separated from the nitrating mixture in the usual manner. Separation from the spent acid will require from about seventeen to twenty-one minutes. The nitrated products, after washing with water and alkaline solution in the usual manner, will have a pH value of (say) 7.0 to 7.1. The water

content will be about .38%-.76%. The dry weight of the product from about a hundred parts of the mixture of glycerine-diglycerine and toluene will be about 235 to 240 parts or a yield of about 94 to 97%. The nitrogen content of the finished product will be about 17%.

It will now be understood that the method in accordance with this invention involves, broadly, the simultaneous nitration of glycerine, glycol or the like and toluene for the production of an explosive involving nitrated glycerine, glycol or the like and nitrated toluene, and that more particularly the invention involves the procedure to effect the nitration comprising the introduction of glycerine, glycol or the like into a nitrating mixture, and the simultaneous introduction of toluene into the nitrating mixture, the toluene being desirably introduced into the nitrating mixture after about one-third of the glycerine, glycol or the like has been introduced and the toluene being introduced during the introduction of a second third of the glycerine, glycol or the like.

It will be understood that where, in the claims hereto appended, glycerine is specified, it is intended to include diglycerine, glycerin-glycol-sugar mixtures, glycerin-sugar mixtures, glycol, or the like, as equivalents for glycerine.

Having now fully described our invention, what we claim and desire to protect by Letters Patent is:

1. The method of producing an explosive which includes introducing a quantity of glycerine into a nitrating mixture, then introducing a quantity of glycerine and a quantity of toluene simultaneously into the nitrating mixture, and finally introducing a further quantity of glycerine into the nitrating mixture.

2. The method of producing an explosive which includes introducing about 30-40 parts of glycerine into a nitrating mixture, then introducing about 30-40 parts of glycerine into the nitrating mixture while separately introducing about 7 parts of toluene into the nitrating mixture, and finally introducing about 30-40 parts of glycerine into the nitrating mixture.

In testimony of which invention, we have hereunto respectively set our hands at Wilmington, Delaware, on this 19th day of September, 1929, and at Kenvil, New Jersey, on this 3rd day of September, 1929.

CORNELL H. CORDIE.  
WILLARD DE C. CRATER.